

(No Model.)

P. LANGHAMMER.

LEAD PIPE.

No. 258,082.

Patented May 16, 1882.



*Fig. 2.*



WITNESSES

Charles R. Searle,  
H. A. Johnston.

INVENTOR

Paul Langhammer  
by his attorney  
Thomas D. Stetson.

# UNITED STATES PATENT OFFICE.

PAUL LANGHAMMER, OF DENVER, COLORADO, ASSIGNOR TO HIMSELF AND  
CHARLES SIEDLER, OF JERSEY CITY, NEW JERSEY.

## LEAD PIPE.

SPECIFICATION forming part of Letters Patent No. 258,082, dated May 16, 1882.

Application filed April 1, 1881. (No model.)

To all whom it may concern:

Be it known that I, PAUL LANGHAMMER, a citizen of the United States, residing at Denver, in the county of Arapahoe, State of Colorado, have invented certain new and useful Improvements Relating to Lead Pipes, of which the following is a specification.

There have been various efforts to produce an insoluble stratum on the interiors of lead pipes. So far as my knowledge extends all have been failures previous to mine. I subject the lead pipe immediately after its manufacture, and while it retains its original heat, to treatment which changes a considerable thickness of the inner portion of the metal and puts it in a condition not liable to be in the least affected by any kind of water or other ordinary fluid which may pass through or stand in it. The pipe after my treatment may be bent and rebent to the fullest extent ever required in putting the pipe in use, and the condition of the interior and of the whole pipe remains unaffected for an indefinite period. My process can be worked in the large way with little labor or skill.

The following is a description of what I consider the best means of carrying out the invention.

The accompanying drawings form a part of this specification.

Figure 1 is a general section of the entire apparatus, certain portions being in elevation. Fig. 2 is on a larger scale. It is a cross-section of my lead pipe after being treated.

Similar letters of reference indicate like parts in the figures.

M' is the main body of the lead pipe. M<sup>2</sup> is my insoluble layer, which is formed on the interior thereof. I will designate the previous condition of the pipe, when necessary, by the single letter M.

A is a car supporting a length of freshly-made lead pipe, M, in its properly-coiled condition, ready for packing and transportation, except that the ends are straightened so as to stand a little out from the coil. I temporarily connect by strong clamps I the two stop-cocks J J' and hose K K'. The hose K leads away to a tank. (Not represented.) The hose K' leads to a drain for waste water. To the lower

end of the coil I correspondingly attach by clamps H two stop-cocks, G G', and two hose, F F'. The hose F leads from a strong boiler, E, in which is stored a solution, to be described farther on. It is at a temperature of about 257° Fahrenheit and the corresponding pressure. The hose F' leads from the street-main or from a suitable elevated reservoir, E', supplying pure water.

Operation: I take on the car A the lead pipe M, in a chemically-clean condition, fresh from the dies or apparatus in which it is produced, and, having the ends properly extended, connect the clamps H and I to the respective ends, open the cocks G and J, and provide for keeping the whole at the temperature of 257° Fahrenheit. The solution from the boiler E rapidly fills the pipe M, driving out the air through the hose K. So soon as the dense solution commences to be delivered from K, I close the stop-cock J, and leave the solution under full pressure in the pipe.

It is essential to success that the heat and pressure be maintained for a considerable time. I attain this end and insure that there shall be a change in a portion of the thickness of the lead, beginning at the extreme surface on the inner side and gradually diminishing. This change should be produced to a depth of about one-fourth of the thickness of the pipe, gradually growing less and less as the chemicals under the considerable pressure and high temperature act successively on the several particles or layers of lead from the interior outward. In order to maintain the pressure, it is simply necessary to keep open the cock G; but in order to maintain the temperature for the considerable time required further provisions are necessary.

L is a casing or oven, of masonry or other material, maintained at a high temperature by gases from the boiler-furnace or otherwise. It receives and surrounds the entire car A with its load, a proper door (not shown) being provided to allow the car A and its load to move in and out. This oven holds the temperature to the proper point. If the pipe, in consequence of its being brought too soon from the manufacturing apparatus, possesses too much of its original heat, its temperature is soon

lowered. If, by any chance, its temperature is too low, it is raised by the oven and held to the proper temperature during the considerable time that the treatment is continued. After from ten to fifteen minutes, or when a sufficient time has elapsed so that I am certain that an insoluble condition has been induced in a considerable thickness of the interior of the pipe, I close the stop-cock G and open the stop-cocks G' J, allowing a stream of pure water to flow through the pipe for a sufficient time to force out into a suitable receptacle (not shown) the solution which remains uncombined, after which I open J', close J, and allow the water to flow to waste through the pipe K'. Then I close the stop-cocks G' and J', disconnect the clamps H and I, and move away the car with its pipe and bring another and repeat the round of operations.

The solution which I employ is sulphate of potassium. This is dissolved in water, and forms a nearly or quite saturated solution. The action in the lead pipes combines some of the sulphur with the inner face of the lead, forming insoluble sulphate of lead. The solution which is discharged through the hose K is partly deprived of its sulphur, and is largely a solution of caustic potash. This may be concentrated by boiling and returned to the manufacturer to aid in the production of more sulphate of potassium, or, by the addition of proper elements, may probably be changed at once into a solution of the required strength to be pumped into the boiler E. It will be understood that the first portion of the discharge is allowed to flow through the hose K into the tank, and that after the main portion of the partly-spent solution has been thus discharged the other stop cock, J', is opened, and momentarily the discharge will be through both; but as soon as practicable after the cock J' is open the cock J is closed.

My theory of the chemical reactions occurring in the working of my process may not be important, but I believe that of the three lead sulphides indicated,  $PbS$ , which is highly crystalline,  $Pb_2S$ , which is also crystalline, and the  $Pb_3S$ , which is soft and semi-metallic, my treatment develops the latter instead of either of the former.  $Pb_3S$  is sufficiently insoluble under all ordinary conditions to serve for domestic and manufacturing purposes with all kinds of water which occur in nature, or any other fluids which are likely to be passed through

my pipe in ordinary business. Its superior flexibility allows it to be quite thick without seriously affecting the fitting of the pipe in all the different bends which are required in practice, and its thickness and its intimate union with, and, as I believe, blending into, the metallic part remaining unaffected insure against its ever being detached from the interior of the pipe by bending or other causes.

Modifications may be made. I can use part of the invention without the whole.

I propose in some cases to draw out the car and its load from the oven before the rinsing process; but in such case I effect the rinsing immediately on such removal. I desire to prevent the formation of any considerable thickness of crust on the interior of the pipe, and rely upon the slight change of the solid body of the metal due to the action of small quantities of the solution within the surface of the metal. I prefer the apparatus described.

I believe that the invention may be worked successfully using a solution of sulphide of potassium instead of sulphate. This is especially expedient in cases where the lead contains an unusual proportion of antimony or copper; but I prefer the sulphate, as described, for lead of ordinary purity.

I claim as my invention—

1. The process of filling lead pipe with a solution of sulphate of potassium and holding it therein under pressure at a temperature of about  $257^{\circ}$  Fahrenheit, so as to produce the highly-metalline sulphate composed of four atoms of lead to one of sulphur in the inner and lining portion, as set forth.

2. The apparatus described, having the boiler E, hose F, cock G, clamps H' I, cock J, hose K, and oven L, for subjecting the interior of the pipe M to a solution at high temperature and under pressure, in combination with the reservoir or main E', hose F', cocks G' J', and hose K', for conveniently removing the uncombined particles of the solution, as herein specified.

In testimony whereof I have hereunto set my hand, at New York city, this 23d day of March, 1881, in the presence of two subscribing witnesses.

P. LANGHAMMER.

Witnesses:

M. F. BOYLE,  
CHARLES C. STETSON.